

# United States Patent [19]

Taub

[11] Patent Number: 4,512,824

[45] Date of Patent: Apr. 23, 1985

[54] DYNAMIC ANNEALING METHOD FOR  
OPTIMIZING THE MAGNETIC  
PROPERTIES OF AMORPHOUS METALS

[75] Inventor: Alan I. Taub, Schenectady, N.Y.

[73] Assignee: General Electric Company,  
Schenectady, N.Y.

[21] Appl. No.: 364,299

[22] Filed: Apr. 1, 1982

[51] Int. Cl.<sup>3</sup> ..... H01F 1/00

[52] U.S. Cl. ..... 148/121; 29/605;  
72/128; 148/31.55

[58] Field of Search ..... 148/120, 121, 122, 31.55,  
148/150; 29/605; 72/128

## [56] References Cited

### U.S. PATENT DOCUMENTS

3,990,923 11/1976 Takashina et al. ..... 148/111

|           |        |                          |           |
|-----------|--------|--------------------------|-----------|
| 4,116,728 | 9/1978 | Becker et al. ....       | 148/31.55 |
| 4,249,969 | 2/1981 | DeCristofaro et al. .... | 148/121   |
| 4,262,233 | 4/1981 | Becker et al. ....       | 148/121   |
| 4,284,441 | 8/1981 | Satoh et al. ....        | 148/120   |
| 4,286,188 | 8/1981 | Honsinger et al. ....    | 148/121   |
| 4,288,260 | 9/1981 | Senno et al. ....        | 148/121   |
| 4,311,539 | 1/1982 | Uedaia et al. ....       | 148/121   |
| 4,321,090 | 3/1982 | Datta et al. ....        | 148/31.55 |
| 4,368,447 | 1/1983 | Inomata et al. ....      | 148/31.55 |
| 4,404,047 | 9/1983 | Wilks ....               | 148/150   |

Primary Examiner—John P. Sheehan

Attorney, Agent, or Firm—Paul E. Rochford; James C. Davis, Jr.; James Magee, Jr.

## [57]

### ABSTRACT

The magnetic properties of metallic alloys in amorphous form are optimized in as-formed configurations by the dynamic annealing process of this invention.

17 Claims, 14 Drawing Figures



FIG. 1A



FIG. 1B



FIG. 1C



FIG. 3



FIG. 2



FIG. 4



FIG. 5



FIG. 6



FIG. 7



FIG. 8



FIG. 9



FIG. 11



FIG. 10



**DYNAMIC ANNEALING METHOD FOR  
OPTIMIZING THE MAGNETIC PROPERTIES OF  
AMORPHOUS METALS**

**BACKGROUND OF THE INVENTION**

This invention pertains generally to metallic alloys in amorphous form useful in the construction of electrical and magnetic devices, and more particularly to methods for optimizing the magnetic properties of amorphous metals when formed into configurations such as cores for electrical transformers.

Amorphous metals are principally characterized by a virtual absence of a periodic repeating structure on the atomic level, i.e., the crystal lattice, which is a hallmark of their crystalline metallic counterparts. The non-crystalline amorphous structure is produced by rapidly cooling a molten alloy of appropriate composition such as those described by Chen et al., in U.S. Pat. No. 3,856,513, herein incorporated by reference.

In one such process for producing amorphous metal in commercially practicable lots, the chill-block melt spinning process, a stream of molten metal of appropriate composition is ejected from a crucible onto one or more rapidly moving chill or substrate surfaces and rapidly quenched, i.e., cooling rates on the order of about  $10^4$  to  $10^6$  °C./sec., to form an elongated thin ribbon-like body whose length is appreciably greater than either its width or thickness. Due to the rapid cooling rates, the alloy does not form in the crystalline state, but assumes a metastable non-crystalline structure representative of the liquid phase from which it was formed. Due to the absence of crystalline atomic structure, amorphous alloys are frequently referred to as "glassy" alloys. The quench rates achieved during the rapid quenching and solidification are controlled primarily by the thickness of the ribbon and the effectiveness of the interfacial contact between the substrate and the ribbon.

Depending upon the composition, many unique properties can be obtained in amorphous metals which cannot necessarily be obtained in crystalline metallic alloys. The unique magnetic properties of the amorphous alloys, for example, have attracted considerable attention. As a class, amorphous alloys exhibit higher magnetic permeabilities, i.e., the ratio of magnetic flux density (B) produced in a medium to the magnetizing force (H) producing it, than crystalline alloys. Also, as a class, the amorphous alloys are more magnetically "soft", i.e., exhibit lower coercive forces (H<sub>c</sub>), than crystalline alloys. The unique magnetic properties of amorphous metallic alloys have led to proposals that magnetically soft amorphous metallic alloys be substituted for presently used magnetically soft crystalline metallic alloys in a variety of devices and applications. Candidates for the substitution include, for example, transformers of various sizes and types in which the cores are generally presently made of grain-oriented 3% silicon steels, magnetic delay lines, magnetic recording heads, and transducers such as stress and strain gauges.

Unfortunately, the highly desirable soft magnetic properties of amorphous metallic alloys are highly stress sensitive and deteriorate rapidly with increasing stress. This stress sensitivity is potentially limiting for many applications envisioned for amorphous metals and is particularly so for transformers and the like wherein the typically thin ribbon-like amorphous metal is wound on itself layer upon layer to form the core.

In general, stresses in amorphous metals may be classified as either residual or applied. Residual stresses typically result, at least in part, from the rapid cooling rates encountered during formation of the amorphous metal, as, for example, by the above-discussed chill-block melt spinning process. Due to their origin, those residual stresses are frequently referred to as "cast-in" or "quenched-in" stresses.

Applied stresses are those which result from the direct application of a load or are present due to the configuration to which the ribbon has been made to conform, e.g., ribbon wound on itself to form a transformer core. Both types of stresses are considered equivalent insofar as they are detrimental to the magnetic properties of amorphous alloys.

It is known that stresses in amorphous metals may be relieved by isothermal annealing. The maximum temperature allowable is that temperature at which the metastable glassy alloy begins to transform to its equilibrium crystalline state, i.e., the crystallization temperature ( $T_x$ ). The desirable soft magnetic properties of amorphous metals generally degrade rapidly with the onset of crystallization. Data in the literature indicates, however, that some crystallinity, i.e., on the order of about 2% or less, may be beneficial in some applications especially at frequencies greater than about several hundred Hertz.

The crystallization temperature is a function of several variables including, for example, local variations in composition. Unlike the melting point of a pure metal, the crystallization temperature of an amorphous alloy is generally not a fixed quantity and may be influenced by the method used in its determination. Frequently, the crystallization temperature is determined by the method known as Differential Scanning Calorimetry (DSC) and then most frequently at a scanning or heating rate of 20° C./min. Another technique commonly used with the DSC method is to determine  $T_x$  at several scanning rates and report as  $T_x$  the value determined by extrapolating to zero scanning rate. All too frequently, however,  $T_x$  is reported without reference to its method of determination.

Therefore, due to the uncertainties in the determination of  $T_x$ , it is preferable to anneal at temperatures sufficiently below  $T_x$  to ensure that crystallization does not occur. As the stress relief annealing temperature decreases below  $T_x$ , however, increases in annealing time, which are undesirable from a manufacturing productivity standpoint, are required. Excessive annealing times also promote brittleness.

The balance between isothermal annealing time and temperature is particularly critical and difficult to control in applications in which the ribbon has been formed to shape, e.g., wrapped to form a transformer core, prior to the anneal. When the core is subsequently annealed, each layer of the core experiences a different temperature-time history as the heat diffuses inwardly, thus yielding a non-uniform product. Further, once the ribbon has been annealed in a configured shape, it may not be reconfigured to a different shape without reintroducing detrimental stresses.

Various methods of stress relieving a moving ribbon have emerged in response to the difficulties experienced with batch isothermal annealing. One such method is taught by Senno et al. in U.S. Pat. No. 4,288,260, which is herein incorporated by reference. The method of Senno et al. principally comprises the continuous transfer of amorphous alloy ribbon between two stations

over at least one heating body situated in-between the two stations such that at least one surface of the ribbon directly contacts the heating body during transfer.

Senno et al. set forth ranges for the rate at which the ribbon should be transferred over the heated body for which temperature ranges are also set forth. Generally, at a fixed transfer rate, the magnetic properties of the ribbon treated by the method of Senno et al. improve with increasing temperature of the heating body, but the improvement appears to be limited by the onset of crystallization. As the duration of the heat treatment increases, i.e., transfer rate decreases, the magnetic properties also generally improve. Thus, the magnetic properties of amorphous ribbons treated by the method of Senno et al. improve as the process conditions approach those of isothermal annealing. No critical inter-relationship between transfer rate and the temperature of the heating body is shown. Senno et al. do not attribute any criticality to post-annealing operations, particularly ribbon handling operations, as the annealed ribbon is simply collected on a take-up reel.

Another method is taught by Satoh et al. in U.S. Pat. No. 4,284,441, which is also incorporated herein by reference. By the method of Satoh et al., internal stresses in a thin strip or ribbon of amorphous alloy are alleviated and the soft magnetic properties improved by alternately imparting tensile and compressive forces to the thin strip while the thin strip is maintained at a temperature within the range in which no deterioration of mechanical properties is induced. The alternate impartation of tensile and compressive forces to the thin strip of amorphous alloy is accomplished by causing the thin strip to be moved over at least one roller having a fixed radius of curvature. The treated ribbons are collected on take-up spools or bobbins and it is generally taught that the diameter of the bobbin should be greater than the diameter of any of the rollers used in the process. Satoh et al. provide only general teachings about such variables as roller diameter, the range of heating temperature and the travelling speed of the ribbon.

Satoh et al. further teach that the internal stress of the thin strip of amorphous alloy can be alleviated merely by moving the unheated thin strip at least once over a roller in such a manner that the ribbon surface opposite to the surface which came into contact with the chill surface is held in contact with the roller. Satoh et al. also teach that a magnetic iron core having good magnetic properties can be fabricated from ribbon treated by their method by rolling the treated ribbon into a core in such a way that the inside surface of the core is formed by the ribbon surface opposite to the surface which was in contact with the chill surface. That teaching is given without any regard to the variable stresses which might thereby be introduced as the radius of the wound object changes.

#### SUMMARY OF THE INVENTION

Although the prior art teaches methods of both static and non-static stress relief annealing of amorphous metals to improve magnetic properties, I have found that the prior art does not fully appreciate the metallurgical phenomena which determine the relief of stresses and the development of optimum soft magnetic properties in amorphous metals. I have further found that the prior art methods are not capable of producing amorphous metals that are substantially completely stress-relieved and, therefore, do not have optimized soft magnetic properties. Therefore, there existed, prior to my inven-

tion, a lack of understanding and methodology for optimizing the soft magnetic properties of amorphous metals particularly when those amorphous metals are deformed and configured into useful shapes such as the cores of electrical transformers.

I have found that the competing material processes of flow and structural relaxation must be accounted for in order to optimize the development of soft magnetic properties in amorphous metals. Specifically, flow must be maximized and structural relaxation must be minimized. Once that state is obtained with the amorphous metal in its final shape, that state must be preserved.

Briefly, the process that I have developed based on my newly found understanding of the material processes of amorphous metals, which I have termed dynamic annealing, involves (a) forming a single thickness of the amorphous metal, typically in the form of a ribbon-like body, to a predetermined final shape or configuration; (b) rapidly heating the thusly formed amorphous metal so as to maximize flow and minimize structural relaxation by heating to the highest peak temperature at the most rapid heating rate attainable subject to the proviso that substantially no crystallization is induced in the amorphous material in the time required during this step to reduce the stresses in the amorphous material by at least 90%, and preferably by at least 95%, of the stresses present in the amorphous material immediately prior to initiation of this heating step; and (c) rapidly cooling the amorphous metal while maintaining the formed shape.

Since the process is preferably performed on a ribbon, moving continuously or incrementally, each increment of the ribbon-like body is essentially given a separate time-temperature stress relief cycle at the instantaneous shape which it will have in the final product which tailors it to a final substantially stress-free configuration having optimized soft magnetic properties. Typically and preferably the rate of rapid heating is equal to or greater than about 300° C./min which is a rate obtainable with beams of energized particles and heat beams, such as those emanating from electron beam devices, line heaters and laser devices, or by resistance self-heating.

The products of my invention are broadly described as discrete bodies which are substantially uniformly stress-free throughout and have optimized soft magnetic properties which are also substantially uniform throughout comprised of a plurality of layers or thicknesses of amorphous metallic material which have been dynamically annealed by the method of the invention to render the material in the as-formed body substantially stress-free, i.e., relieved of at least 90%, and preferably 95% or more, of the initial stress present in the material before dynamic annealing.

#### BRIEF DESCRIPTION OF THE DRAWINGS

The practice of my invention may be more fully understood and its features and advantages more readily appreciated by the detailed description provided hereinbelow with reference to the appended FIGURES wherein, briefly:

FIG. 1A is a schematic representation of the state of stress in a bent segment of a thin ribbon-like body;

FIG. 1B is a schematic representation of the state of stress in a segment of a thin ribbon-like body at an intermediate time during a stress-relief anneal showing partial relief of the internal stresses;

FIG. 1C is a schematic representation of the state of stress in the ribbon-like body of FIG. 1B following completion of the annealing treatment;

FIG. 2 is a log-log graph of the stress relief fraction in bending versus annealing time for  $Pd_{77.5}Cu_6Si_{16.5}$  amorphous metal ribbons annealed at  $498^\circ$  and  $523^\circ$  K.;

FIG. 3 is a graph of the logarithm of viscosity versus inverse temperature which shows schematically the formation of the amorphous metallic state and wherein the phenomenon of structural relaxation is also schematically represented;

FIG. 4 is a graph of temperature versus time, whereon several isoflow and isostructural contours are plotted, which illustrates the interaction between flow and structural relaxation;

FIG. 5 shows schematically an elementary apparatus suitable for the practice of the dynamic annealing process of the invention;

FIG. 6 shows schematically another embodiment of apparatus suitable for the practice of the dynamic annealing process of the invention wherein the amorphous metallic ribbon is dynamically annealed at a location remote from the final product;

FIG. 7 shows schematically a further embodiment of apparatus suitable for the practice of the process of the invention employing two sequentially operated stations for producing dynamically annealed ribbon suitable for forming, for example, a wound substantially stress-free product of substantially rectangular cross-section;

FIG. 8 is a graph of a typical temperature-time thermal cycle produced in amorphous metallic ribbon when dynamically annealed by the apparatus of FIG. 6 using a focussed heat source;

FIG. 9 is a graph of the direct current magnetic properties of  $Fe_{81.5}B_{14.5}Si_4$  amorphous metallic ribbon dynamically annealed by the method of the invention on the apparatus of FIG. 6 and by conventional isothermal annealing;

FIG. 10 shows schematically a portion of apparatus for annealing amorphous metallic ribbons using heated block contact heating means;

FIG. 11 is a graph of percent stress-relief versus feed rate for  $Fe_{81.5}B_{14.5}Si_4$  amorphous metallic ribbons annealed at several temperatures using the apparatus of FIG. 10; and

FIG. 12 is a semi-logarithmic graph comparing alternating current magnetic properties at 14 kilogauss of amorphous metallic ribbon annealed by conventional isothermal and contact block heater mean and by the dynamic annealing method of the invention as a function of heating rate.

#### DETAILED DESCRIPTION OF THE INVENTION AND PREFERRED EMBODIMENTS

There are two factors which govern the relief of stresses in amorphous metals. Those two factors are flow and structural relaxation. Flow refers to homogeneous deformation in response to stress. Flow, in turn, consists of two components, i.e., viscoelastic or irreversible flow and anelastic or reversible flow, which are described in more detail below.

A stress pattern such as is found in a bent or coiled segment of amorphous metal ribbon is shown in FIG. 1A. As discussed above, the total stress will consist of at least an applied component due to the bent shape of the ribbon and quite typically a residual component due to quenched-in stresses. The stress pattern of FIG. 1A

varies linearly through thickness,  $x$ , of ribbon segment 20 from maximum compressive at inner surface 22 to zero at neutral axis 26, to maximum tensile at outer surface 24. In the FIGURES and following discussion, the tensile and compressive stresses are expressed in terms of the absolute value of the equivalent shear stress  $|\tau|$ .

If amorphous metal ribbon 20 is heated to an elevated temperature,  $T_a$ , above room temperature, i.e., annealed, the amorphous metal of ribbon 20 will flow in response to the stress  $|\tau|$ . According to classical prior art theory, such an annealing process will result in a stress-free ribbon if conducted for a sufficient time. The higher the annealing temperature is above room temperature, the less time will be required for stress relief.

In contrast to the classical theory, I have found that for amorphous metals there is a threshold value of stress,  $\tau_o$ , below which the stresses will not decay or relieve. As ribbon 20 is annealed, that portion of ribbon 20 subjected to an absolute stress of  $|\tau| > \tau_o$  exhibits flow while those portions of ribbon 20 subjected to an absolute stress of  $|\tau| < \tau_o$  exhibit no flow as is shown schematically in FIG. 1B. Ultimately, the stress distribution shown in FIG. 1C is obtained. Annealing at high temperatures has the advantage of reducing the residual stress pattern since  $\tau_o$  decreases with increasing temperature. However, as discussed above, the closer the annealing temperature  $T_a$  is to  $T_x$ , the crystallization temperature, the more likely is the possibility that detrimental crystallization will occur.

A model which I have developed which provides a complete description of the kinetics of stress relief in amorphous alloy ribbons bent to an initial fixed radius,  $r_o$ , and incorporates the threshold value  $\tau_o$  is as follows:

$$\left[ 1 - \frac{r_o}{r(t)} \right] = K + [1 - K] \left[ 1 + \frac{\dot{\eta}t}{\eta_o} \right]^{-E/3\dot{\eta}} \quad (1)$$

where

$r(t)$ =unconstrained natural radius of curvature of the ribbon as a function of time,  $t$ ;

$\tau_{max} = \tau_i$ =maximum shear stress at  $t=0$ ;

$\tau_o$ =threshold value of the equivalent shear stress;

$E$ =elastic modulus (Young's Modulus);

$\eta_o$ =viscosity at  $t=0$ ;

$\dot{\eta}$ =rate of viscosity increase with time, and

$$K = \frac{3}{2} \cdot \frac{\tau_o}{\tau_{max}} - \frac{1}{2} \left( \frac{\tau_o}{\tau_{max}} \right)^3$$

The correspondence between the model and the stress relief of an as-cast  $Pd_{77.5}Cu_6Si_{16.5}$  amorphous alloy ribbon at two annealing temperatures,  $498^\circ$  and  $523^\circ$  K., is shown in FIG. 2. The solid symbols represent actual data points and the solid lines represent the model of equation (2). The degree of stress relief increases with both testing time and testing temperature and asymptotically approaches the x-axis at long annealing times. The difference between the asymptotic value and 100% stress relief is due to  $\tau_o$ .

The second factor, structural relaxation, occurs in parallel with flow during stress-relief annealing. I have found that this second factor must also be accounted for

in order to optimize the stress-relief annealing of amorphous alloys. The origin of structural relaxation may be explained with reference to FIG. 3.

When a molten glass-forming metallic alloy is quenched rapidly enough to avoid crystallization, the equilibrium liquid properties are extrapolated into the metastable regime below the melting temperature,  $T_m$ , as shown schematically in FIG. 3. As the temperature decreases below  $T_m$  during this quench, the atomic mobility is sufficient to permit the atomic structure of the alloy to continuously adopt equilibrium configurations. This rearrangement continues until the region of the glass transition temperature,  $T_g$ , is reached. At some temperature near  $T_g$ , the atomic configuration becomes "frozen" because the resistance to atomic motion, i.e., the viscosity, is large enough to restrict structural rearrangement. That is, the time required for the atoms to adopt their equilibrium configurations is greater than the quenching time scale, so the alloy structure deviates from equilibrium. This deviation is shown schematically by curve A of FIG. 3. This curve represents the isoconfigurational, i.e., constant structure, properties of the alloy. In contrast, curve D shows the behavior of the same alloy quenched at a much slower rate and solidified directly to the crystalline state.

Subsequent heat treatment of the glassy alloy at temperatures below  $T_g$  allows the atomic structure to approach its equilibrium configuration. Significant shifts of the isoconfigurational curves toward the equilibrium curve, as shown schematically by curves B and C of FIG. 3, have been observed for anneals at the same temperatures and times used in stress relief anneals.

Structural relaxation is, therefore, an unavoidable consequence of stress relief annealing. This has an important effect on the properties of the amorphous metal. First, the viscosity increases, i.e., the atomic mobility decreases, as just described. This increase in flow resistance has been associated with embrittlement of the alloy. Perhaps more important for soft magnetic applications is the interaction of the structural relaxation with the flow of these materials and, more specifically, the viscoelastic and anelastic components discussed above since those components interact with the material to produce a magnetic anisotropy.

For positive magnetostriction materials, such as the alloys proposed for transformer applications, flow along the ribbon length produces an anisotropy perpendicular to the lengthwise ribbon axis which is detrimental to transformer performance. It appears that the anelastic flow is primarily responsible for the induction of this anisotropy. Structural relaxation is important because of its effect on the flow mechanism. Structural relaxation has been shown to dramatically decrease the viscoelastic strain rate. Therefore, it is expected that flow in a non-relaxed glass, i.e., a low viscosity glass, will have a higher ratio of viscoelastic to anelastic flow than in a relaxed glass, i.e., a high viscosity glass. Thus, if a large amount of structural relaxation occurs during a stress relief anneal, it would be expected that a larger percentage of the flow would be anelastic than if a small amount of structural relaxation occurred. This, in turn, would lead to a larger induced detrimental anisotropy.

I have found that mere knowledge of the phenomena of flow and structural relaxation in amorphous metals is inadequate to enable one to optimize the stress relief and magnetic properties of amorphous metals. As I have discovered, it is necessary to understand the interaction

between flow and structural relaxation in order to optimize the stress relief of amorphous metals. To explain that newly found understanding, I have derived FIG. 4.

It is known that the temperature dependence of the viscosity for a constant structure,  $\eta_0$ , and the rate of viscosity change with temperature,  $\dot{\eta}$ , may be closely approximated by:

$$\eta_0 = N_0 e^{Q_{iso}/kT} \quad (2)$$

and

$$\dot{\eta} = \dot{N}_0 e^{Q_{\dot{\eta}}/kT} \quad (3)$$

respectively, where

$N_0$ =pre-exponential material parameter;  
 $N_0$ =pre-exponential material parameter;  
 $Q_{iso}$ =activation energy for flow at constant structure;  
 $Q_{\dot{\eta}}$ =activation energy for rate of viscosity increase;  
 $k$ =universal gas constant in appropriate units; and  
 $T$ =absolute temperature (°K)

Equations (2) and (3) may be combined with equation (1), which expresses the relationship between stress and time at a constant temperature, to yield the following equation

$$t = [C^{-3\dot{\eta}/E} - 1] \frac{N_0}{\dot{N}_0} e^{(Q_{iso} - Q_{\dot{\eta}})/kT} \quad (4)$$

which expresses the relationship between time and temperature of an amorphous metal flowing at a constant stress where

$$C = \frac{\tau(t) - \tau_0}{\tau_i - \tau_0}$$

with the remaining terms being defined as above.

The solid curves of FIG. 4 represent the solution of flow equation (4) for the various values of  $\tau(t)/\tau_i$  shown. As the value of  $\tau(t)/\tau_i$  decreases, the amount of flow increases.

Equations (3) and (4) may be combined to yield the following equation:

$$\ln \frac{t}{t_0} = \frac{Q_{iso} - Q_{\dot{\eta}}}{k} \left( \frac{1}{T} - \frac{1}{T_0} \right) \quad (5)$$

wherein  $t$  is time,  $t_0$  is an arbitrary reference time, and  $T_0$  is an arbitrary reference temperature with the remaining terms as previously described, which permits the plotting of the dashed isostructural contours on FIG. 4. Referring back to FIG. 3, the initial state of an as-cast amorphous alloy is represented by curve A. During annealing, the isoconfigurational curve will shift towards the equilibrium curve as shown by intermediate curves B and C. In FIG. 4, the structural relaxation is represented by the shift of the dashed curves toward higher values of  $\eta(T_0)$ . The parameters used in Equations (4) and (5) to construct FIG. 4 were:  $E=100\text{GPa}$ ,  $\tau_0=15\text{MPa}$ ,  $Q_{iso}=220\text{kJ/mole}$ ,  $Q_{\dot{\eta}}=35\text{kJ/mole}$ ,  $N_0=1\times 10^{-8} \text{ Pa-s}$ , and  $\dot{N}_0=2\times 10^7 \text{ Pa}$ . These are typical values for many amorphous alloys.

FIG. 4 may be used to compare the relative rates and effects of stress relief and structural relaxation. Two

points of constant stress relief fraction are marked on FIG. 4 as points 1 and 2. Point 1 is for an isothermal anneal performed at 563° K. for 300 seconds. Point 2 is for an anneal at a lower temperature of 540° K. for a longer time of 3100 seconds. In both cases, the stress has been relieved to the same value of  $\tau(t)/\tau_i$ , i.e., 30%, which represents that 70% of the stresses initially present have been relieved. Point 1, however, intersects an isothermal contour that corresponds to a lesser degree of structural relaxation (3.9) than the corresponding 10 isostructural contour for point 2 (6.9).

Since lower degrees of structural relaxation reduce the opportunity for detrimental anelastic flow and concomitant detrimental induced anisotropy to occur, and also reduce the opportunity for embrittlement, it is expected that an amorphous metal stress relieved at the conditions of Point 1 would have better magnetic properties and be less brittle than the same metal stress relieved at the conditions of Point 2. My FIG. 4 thus explains why isothermal annealing or annealing at slow 20 feed rates and low temperatures is undesirable, i.e., by the time an adequate amount of flow has been achieved to effect the desired amount of stress relief, too much detrimental structural relaxation has occurred.

Since the curves of FIG. 4 slope steeply upward at small values of time, the only way to obtain the benefits of minimized structural relaxation is to heat as rapidly as possible to the annealing temperature to minimize the number of isoconfigurational contours intersected. Heating rate, however, is not the only variable involved. Another relevant, but not independent, factor is crystallization. For the purposes of my invention, it is desirable that substantially no crystallization occur in the amorphous metal during dynamic annealing in order that soft magnetic properties are optimized. Substantially no crystallization means that the amorphous metal contains no more than about 2% crystallinity by volume as measured by such analytical techniques as X-ray and electron diffraction and light microscopy, or combinations thereof, or as may be inferred from magnetic measurements.

The crystallization behavior of amorphous metals is a function of the crystallization temperature,  $T_x$ , which increases with heating rate,  $dT/dt$ , and the time required for crystallization,  $t_x$ , which decreases with increasing annealing temperature,  $T_a$ . Thus, given the criteria that substantially no crystallization is to be induced in the amorphous metallic alloy during annealing, there are three interrelated variables that must be satisfied, i.e., the annealing temperature ( $T_a$ ), the time ( $t_a$ ) at the annealing temperature, and the heating rate to the annealing temperature ( $dT_a/dt$ ). Those variables are subject to the additional condition that the annealing time and annealing temperature must be sufficient to provide adequate relief of the stresses and that once 55 stress relieved no permanent stresses are reintroduced into the material. Lastly, once the objectives are obtained, it is necessary to cool sufficiently rapidly from the annealing temperature to prevent any significant additional structural relaxation from occurring and/or to prevent any additional significant crystallization, if any, to the limit of no more than about 2% by volume, from occurring.

The dynamic annealing apparatus shown schematically in FIG. 5 was built in order to implement my above-discussed novel discoveries about the stress relief of amorphous metals. In the apparatus of FIG. 5, amorphous metal ribbon 20 of width,  $W$ , and thickness,  $x$ , is

pulled under constant tension from supply spool 30 past guide roller 31 and wrapped around core form 32. Heat from concentrated heat source 34 is directed at a single thickness of ribbon 20 after it has attained its final configuration which, as shown, is a spiral of ever-increasing diameter. Ribbon 20 is then rapidly cooled by means 36 to prevent heat buildup in previously treated and wrapped layers, e.g., layers 20', 20'', and 20''. It is essential that ribbon 20 not be heated until after it has reached its final configuration; otherwise, structural relaxation will commence before all the winding stresses have been applied thus lessening the discovered advantages of my invention.

Source 34 preferably provides heat in the form of beam 38 in order to attain heating rates as close as possible to a theoretically preferred infinite heating rate. Suitable sources 34 include, for example, devices which emit electron beams, laser beams, and radiant heat beams. It is also contemplated that means employing direct contact with ribbon 20, such as resistance self-heating through a pair of appropriately situated contact points or probes (not shown), will also provide heating rates sufficiently rapid to enable realization of the benefits of my invention. Additionally contemplated are fluid heating media such as a plasma and a molten salt bath.

Cooling means 36 supplies a jet 40 of a cooling medium, such as air or an inert gas like nitrogen, to ribbon 20 immediately after ribbon 20 exits the area of impingement of beam 40. This cooling serves to "freeze" the as-annealed stress-free structure in ribbon 20 preventing any further significant additional structural relaxation and minimizes the detrimental passage of heat into previously annealed layers 20' and 20''. The use of non-gaseous jets 40, such as streams of water or other suitable liquid quenchants, is also contemplated.

Following rapid heating and rapid cooling while at the final shape, annealed and stress-relieved ribbon 20 is subsequently wound or wrapped layer upon layer about core form 32 to produce product 42. Typically, core form 32 may be circular or polygonal in cross-section and may be solid or hollow. The length of product, or discrete body 42, measured perpendicular to its cross-sectional area, is equal to the width,  $W$ , of ribbon 20. More than one body may be wound, one adjacent to the next along the length of the core form, on the same core form. Although wound on a core form, the final products may or may not have the core form present.

Thus, the products 42 of the invention may generally be described as discrete bodies which are substantially uniformly stress-free throughout having been formed from a plurality of layers or thicknesses of amorphous metallic ribbon, successively wrapped one on top of the other, which have been dynamically annealed by the method of the invention to render the ribbon as-wrapped substantially stress-free, i.e., relieved of at least 90%, and preferably 95% or more, of the initial stresses present in the ribbon in the unwrapped state. As will be developed in greater detail below, the bodies will also have optimized soft magnetic properties which are substantially uniform throughout by reason of the dynamic annealing process and their substantially uniform stress-free state throughout.

As will be appreciated by those skilled in the transformer manufacturing arts, the apparatus of FIG. 5, as well as the other apparatus described herein, may also be adapted to coat ribbon 20 with an insulating material or to interleave ribbon 20 with an insulating material

prior to final wrapping around core form 32. Further, the apparatus described herein can be equipped to provide means for applying a magnetic field to the ribbon during dynamic annealing to further enhance the magnetic properties of amorphous metallic ribbon treated by the method of my invention.

Another apparatus suitable for the practice of my invention is that shown in FIG. 6. The apparatus of FIG. 6 is generally similar to the apparatus of FIG. 5 and like components are similarly numbered. The apparatus of FIG. 6 comprises additionally guide rollers 50, 52 and 54. In the apparatus of FIG. 6, the rapid heating and rapid cooling of ribbon 20 takes place as ribbon 20 traverses the exterior surface of drum or roller 56 and subsequently passes over roller 54 to be wound upon core form 32. The principal advantage of the apparatus of FIG. 6, compared to the apparatus of FIG. 5, is that heating by beam 38 takes place in a manner such that the heat from beam 38 is positively restricted to a single thickness of that segment or increment of ribbon 20 being treated and cannot diffuse into previously annealed and wrapped layers of the ribbon. A similar effect could be obtained in the apparatus of FIG. 5 by placing a fixed insulating member (not shown) beneath that portion of ribbon 20 upon which beam 38 impinges to separate it from the previously dynamically annealed ribbon previously wrapped on core form 32.

Fixed or rotatable drum or roller 56 is also preferably designed to be adjustable so that its instantaneous diameter during heat treatment of ribbon 20 by beam 38 and jet 40 is equal to the diameter, curvature or configuration which ribbon 20 will have when coiled about core form 32 on top of the previously wrapped layers. Guide roller 54 should have a diameter sufficiently large such that the passage of annealed and stress-relieved ribbon 20 thereover will not introduce any plastic strains into ribbon 20.

The apparatus of FIG. 7 illustrates the use of the method of my invention to produce product 42 having a substantially rectangular cross-section. Again, elements of the apparatus of FIG. 7 which are identical to the elements described in conjunction with the apparatus of FIGS. 5 and 6 are similarly numbered. In the apparatus of FIG. 7, amorphous metal ribbon 20 leaves spool 30, passes over guide roller 50 and across platen 60 at dynamic annealing station 70 whereat those segments which will be straight in final product 42, e.g., segments or increments 62 and 64 are dynamically annealed by rapidly heating by means of beam 38 from device 34 and subsequently rapidly cooled by means of

TABLE I

| SPECIMEN | HEATER<br>VOLTS | FEED<br>RATE<br>(cm/min)      | T <sub>peak</sub><br>(°C.) | STRESS                       |                           | MAGNETIC PROPERTIES |                                         |                 |           |
|----------|-----------------|-------------------------------|----------------------------|------------------------------|---------------------------|---------------------|-----------------------------------------|-----------------|-----------|
|          |                 |                               |                            | HEATING<br>RATE<br>(°C./min) | RELIEF<br>FRACTION<br>(%) | DC                  |                                         | AC @ 14 k gauss |           |
|          |                 |                               |                            |                              |                           | Hc<br>(mOe)         | B <sub>1</sub> /B <sub>100</sub><br>(%) | mWatts<br>Lb    | mVA<br>Lb |
| A1       | 230             | 4                             | 448                        | 240                          | 100                       | 33                  | 80                                      | ND              | ND        |
| A2       | "               | 8                             | 436                        | 458                          | 100                       | 33                  | 88                                      | 128             | 269       |
| A3       | "               | 18                            | 398                        | 924                          | 96                        | 28                  | 84                                      | 117             | 657       |
| A4       | "               | 26                            | 350                        | 1300                         | 93                        | 33                  | 74                                      | 112             | 2500      |
| A5       | "               | 34                            | X                          | X                            | 90                        | 35                  | 67                                      | 119             | 5600      |
| A6       | "               | 53                            | X                          | X                            | 68                        | 45                  | 59                                      | ND              | ND        |
| A7       | N/A             | None<br>Isothermal<br>(2 hrs) | 365                        | 10-15                        | 100                       | 63                  | 77                                      | 154             | 1200      |
| A8       | N/A             | None<br>Isothermal<br>(2 hrs) | 345                        | 10-15                        | 100                       | 43                  | 71                                      | 170             | 3100      |
| A9       | N/A             | None<br>As-Cast<br>Straight   | N/A                        | N/A                          | 0                         | 100                 | 48                                      | ND              | ND        |
| A10/A11  | N/A             | None<br>As-Cast               | N/A                        | N/A                          | 0                         | 50-53               | 57-60                                   | ND              | ND        |

jet 40 from cooling means 36. Those segments of ribbon 20 which will be located at the rounded corner segments in final product 42, e.g., segments or increments 66 and 68, are dynamically annealed at station 72 by means of beam 38' from device 34' and cooled by jet 40' from cooling means 36' as those segments pass over adjustable drum or roller 56. Suitable control means (not shown) are provided to suitably sequence the dynamic annealing apparatus at stations 70 and 72 and suitably adjust the diameter of roller or drum 56.

In order to further teach the practice of my invention, and to compare the magnetic properties of amorphous metal ribbons stress relieved by the dynamic annealing method of my invention to those stress relieved by methods of the prior art, the following illustrative, but not limiting, examples and discussion are herewith provided.

## EXAMPLE I

Using the apparatus of FIG. 6, wherein heat source 34 was a quartz line heater manufactured by Research, Inc., which emitted a focused beam of heat 38, a series of Fe<sub>81.5</sub>B<sub>14.5</sub>Si<sub>4</sub> amorphous metal ribbons 41  $\mu\text{m}$  thick by 12 mm wide were dynamically annealed by the method of the invention under the conditions set forth in Table I (Samples A1-A6). Cooling was accomplished by blowing a jet of nitrogen 40 from cooling means 36 in the form of a small diameter tube positioned in close proximity to both ribbon 20 and the location at which beam 38 impinged on ribbon 20.

The ribbons were formed into spirally wound bodies by winding five to fifteen turns or layers about a core form having a diameter of 4.5 cm. Since the diameter of the outermost turn was not significantly different from the diameter of the innermost turn, because only a few layers were wound, it was considered that no stresses would be introduced during winding, thus drum 56 had a fixed and not a variable diameter. Direct and alternating current magnetic measurements were made on the spirally wound bodies with the results also set forth in Table I.

In order to obtain a measurement of the heating rate produced in ribbon 20 by the apparatus of FIG. 6, the outside surface of drum 56 directly beneath the locus of impingement of beam 38 was instrumented with cemented-on foil chromel-alumel thermocouples. Separate measurements made on some ribbons directly instrumented with a 5 mil beaded and flattened chromel-alumel thermocouple spot welded to the face of ribbon

TABLE I-continued

| SPECIMEN | HEATER VOLTS | FEED RATE (cm/min) | T <sub>peak</sub> (°C.) | HEATING RATE (°C./min) | RELIEF FRACTION (%) | STRESS      |                                                      | MAGNETIC PROPERTIES |        |  |
|----------|--------------|--------------------|-------------------------|------------------------|---------------------|-------------|------------------------------------------------------|---------------------|--------|--|
|          |              |                    |                         |                        |                     | DC Hc (mOe) | AC @ 14 k gauss B <sub>1</sub> /B <sub>100</sub> (%) | mWatts Lb           | mVA Lb |  |
| Wound    |              |                    |                         |                        |                     |             |                                                      |                     |        |  |

## KEY:

N/A = Not Applicable

ND = Could Not Be Driven to 14 k gauss

X = Thermocouple Degraded

15

20 opposite to heat source 34 verified that the cemented-on foil thermocouples accurately reflected the heating rate. The spot welded thermocouples additionally provided a measurement of the cooling rate.

A typical temperature-time profile of a ribbon instrumented with a spot welded thermocouple while passing through the impingement zones of beam 38 and cooling jet 40 is shown in FIG. 8. Heating rates as high as approximately 500° C./min were readily obtained. All heating rates reported herein were calculated by subtracting 80° C. from the peak temperature and dividing that quantity by the time required to heat the ribbon 30 from 80° C. to the peak temperature. The heating rate was a function of both heater power (lamp volts) and ribbon feed rate. The peak temperature of the ribbon in the beam impingement zone also changed with those parameters, i.e., the higher the lamp power, the higher 35 the peak temperature, and the faster the feed rate (the less time spent in the beam impingement zone), the lower the peak temperature.

The temperature-time cycle of FIG. 8 shows that a cooling rate approximately as rapid as the heating rate 40 can readily be obtained with the apparatus of FIG. 5. The objective of rapidly cooling the annealed amorphous metal is to ensure that no significant additional structural relaxation and/or no significant additional crystallization, if any, to the limit of no more than about 45 2% by volume, occurs during cooling. The minimum cooling rate required to ensure that substantially no structural relaxation and/or crystallization occurs during cooling can rigorously be calculated by integrating the equations used to derive FIG. 4 with respect to 50 time. However, to a first engineering approximation, for most amorphous metals, the objective can be met by rapidly cooling at a rate of at least about 100° C./min. As used herein and in the claims hereof the term rapidly cooling means cooling at a rate of at least about 100° 55 C./minute.

The direct current (DC) magnetic properties of the ribbons of Example I, dynamically annealed by the method of my invention, are presented in graphical form in FIG. 9. Also presented in Table I and on FIG. 9, are DC magnetic property data for amorphous metallic ribbons of the same composition wound on the same diameter core forms and conventionally annealed isothermally for two hours, exclusive of heat-up and cool-down time, at annealing temperatures of 365° and 345° C. (Samples A7 and A8, respectively). Base-line data for similar amorphous metallic ribbon in the as-cast and uncoiled form and as-cast, but similarly coiled condi-

tion, is also presented in Table I (Samples A9 and A10-A11, respectively).

From Table I and FIG. 9, the ribbons dynamically annealed by the method of my invention are seen to have soft magnetic properties that are considerably improved over those of ribbons stress relieved by prior art isothermal annealing. Further, the degrading effects of over-annealing, which produces crystallization, and the degrading effects of an incomplete stress relief on the soft magnetic properties may also be seen from FIG. 9.

## EXAMPLE II

Two samples (2-1 and 2-2) of Fe<sub>81.5</sub>B<sub>14.5</sub>Si<sub>4</sub> amorphous metallic alloy ribbon 20 were stress relief annealed using the apparatus of FIG. 10 comprising 2" diameter hollow mandrel 80, resistance heated block 82 and ribbon bottom gas cooling jet orifices 84 and ribbon top gas cooling means 86. Those samples were instrumented with a chromel-alumel thermocouple 88 to obtain a measure of the heating rates typical of this type of apparatus. The thermocouples were as described in Example I except for the location which in this example was the outside width surface of the ribbons, but was still the ribbon surface opposite from the heat source. The heating rate data produced are presented in Table II.

Since the samples instrumented with the thermocouples could not be used for magnetic measurements, a second series of samples (Samples D-1 to D-5 of Table II) were stress relief annealed using the apparatus of FIG. 10. The feed rates and block temperature used for this second series and the resulting magnetic property measurements are also presented in Table II.

Using a different and more powerful heating block 82 in mandrel 80 so that higher block temperatures could be obtained, sufficient additional samples of Fe<sub>81.5</sub>B<sub>14.5</sub>Si<sub>4</sub> amorphous metallic alloy were stress relief annealed using the apparatus of FIG. 10 to provide the additional data graphed in FIG. 11. A crystallization temperature, T<sub>x</sub>, of 470° C. was measured for this Fe-B-Si amorphous metallic alloy by Differential Scanning Calorimetry at a scanning rate of 20° C./min. Using that value of T<sub>x</sub> and the teachings of Senno et al., i.e., that for heated block devices T<sub>block</sub> should be in the range of (T<sub>x</sub>-200° C.) ≤ T<sub>block</sub> ≤ (T<sub>x</sub>+50° C.) and the feed rate V should be the range (1 cm/sec) ≤ V ≤ (50 cm/sec), the shaded portion of FIG. 11 was constructed.

Additional experiments similarly conducted, but not shown on FIG. 11, at 583° C. and 7.8 cm/sec feed rate resulted in

TABLE II

| SPECIMEN | FEED RATE (cm/min) | T <sub>block</sub> (°C.) | T <sub>peak</sub> (°C.) | HEATING RATE (°C./min) | STRESS RELIEF FRACTION (%) | MAGNETIC PROPERTIES |                                                      |           |        |
|----------|--------------------|--------------------------|-------------------------|------------------------|----------------------------|---------------------|------------------------------------------------------|-----------|--------|
|          |                    |                          |                         |                        |                            | DC Hc (mOe)         | AC @ 14 k gauss B <sub>1</sub> /B <sub>100</sub> (%) | mWatts Lb | mVA Lb |
| 2-1      | 4.1                | —                        | 439                     | 129                    | —                          | —                   | —                                                    | —         | —      |
| 2-2      | 4.1                | —                        | 515                     | 206                    | —                          | —                   | —                                                    | —         | —      |
| D1       | 8                  | 461                      | —                       | —                      | 100                        | 33                  | 86                                                   | 146       | 2988   |
| D2       | 18                 | —                        | —                       | —                      | 100                        | 30                  | 87                                                   | 143       | 1433   |
| D3       | 23                 | —                        | —                       | —                      | 96                         | 30                  | 86                                                   | 153       | 1967   |
| D4       | 34                 | —                        | —                       | —                      | 96                         | 35                  | 81                                                   | 171       | 1940   |
| D5       | 53                 | —                        | —                       | —                      | 93                         | 35                  | 78                                                   | 185       | 3198   |

86% stress relief and at 600° C. at feed rates of 7.6, 9.6, 15 12.8, and 16.8 cm/sec, resulted in stress relief of 100%, 91%, 73%, and 44%, respectively.

FIG. 11 and the additional experiments thus show that if the feed rates and the stress relief annealing temperatures are selected in accordance with the teachings of Senno et al., the stress relief will be incomplete and, by logical extension, the magnetic properties will not be at their optimum. FIG. 11 and the additional data further show that there are no favorable combinations of the variables of annealing temperature and feed rate, within the ranges taught by Senno et al., that will produce amorphous metallic ribbons which have been stress relieved by at least about 95%.

Using the heating rate data of Samples 2-1 and 2-2 of Table II, an engineering approximation was made of the range of heating rates to be expected for the heating of thin ( $\leq 100 \mu\text{m}$ ) ribbons by contact heating with a hot block such as is done by the apparatus of FIG. 10. Assuming linear heat transfer to the ribbon, it was determined by elementary heat transfer analysis that the heating rate of the ribbon is independent of the rate at which the ribbon passes over the hot block. The analysis further showed that heating rate is a direct function of block temperature.

For a hot block whose temperature,  $T_b$ , is in the range of  $(T_x - 200^\circ \text{C.}) \leq T_b \leq (T_x + 50^\circ \text{C.})$  the analysis 40 and an extrapolation of the data of Table II gave the result that the heating rate,  $dT/dt$ , of a ribbon pulled over the block ranges from about 50° to about 300° C./min for values of the crystallization temperature,  $T_x$ , which are typical for amorphous metals of compositions 45 potentially useful for transformer applications.

Using the above-obtained data and the above-discussed discoveries of my invention, the data of Tables I and II were combined to provide FIG. 12 which is a graph of the alternating current magnetic properties at 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 96

7. The method of claim 1 wherein said forming means are adjustable.

8. The method of claim 1 wherein said method is conducted continuously.

9. The method of claim 1 wherein said method is conducted intermittently.

10. A method for forming a substantially stress-free discrete body, said body being in the form of a plurality of layers of a continuous length of a ribbon-like body of amorphous metallic alloy, comprising the steps of:

(1) traversing a single thickness of said ribbon-like body across at least one forming means to form each predetermined increment of said ribbon-like body to substantially the same configuration it is to have in the completed discrete body;

(2) heating the formed single thickness of said ribbon-like body while in contact with said forming means to the highest peak temperature attainable at a rate greater than about 300° C./min subject to the proviso that substantially no crystallization is induced in said ribbon-like body in the time required during this heating step to reduce the stresses in said material by at least 90% of the stresses present in said amorphous material immediately prior to initiation of said heating;

(3) rapidly cooling the formed single thickness of said ribbon-like body at a rate of at least about 100° C./min while in contact with said forming means; and

(4) thereafter wrapping said ribbon-like body about itself layer upon layer thereby forming said discrete body.

11. The method of claim 10 wherein said stresses in said ribbon-like body are reduced by at least 95% of the stresses present in said ribbon-like body immediately prior to initiation of said heating step.

12. The method of claim 10 wherein said heating is performed by means of an impinging beam from a source selected from the group consisting of a laser beam source, electron beam source, and radiant heat source.

13. The method of claim 10 wherein said heating is performed by means of resistance self-heating.

14. The method of claim 10 wherein said cooling is conducted at a rate greater than about 100° C./min.

15. The method of claim 10 wherein said forming means are adjustable.

16. The method of claim 10 wherein said method is conducted continuously.

17. The method of claim 10 wherein said method is conducted intermittently.

\* \* \* \* \*